

## UNITED STATES PATENT OFFICE.

JEAN H. L. DE BATS, OF EAST ORANGE, NEW JERSEY, ASSIGNOR TO DE BATS METALS COMPANY, OF BLOOMFIELD, NEW JERSEY, A CORPORATION OF NEW JERSEY.

## ALLOY.

No Drawing.

Application filed January 24, 1924. Serial No. 688,303.

To all whom it may concern:

Be it known that I, JEAN H. L. DE BATS, a subject of the Queen of Holland, having declared my intention of becoming an American citizen, residing in East Orange, in the State of New Jersey, have invented certain new and useful Improvements in Alloys, of which the following is a specification.

- 10 This invention relates to alloys designed primarily for the formation of cutting tools and particularly of tools for cutting hard metals, as in lathes, planers, and other machine tools. An alloy designed for such purposes must possess mechanical strength sufficient to resist the reaction of the feed and the pressure of the chip, a sufficient degree of hardness to resist wear under the conditions imposed by high duty, and the ability 20 to retain the qualities of strength and hardness notwithstanding the high temperature developed at the cutting edge under high duty. The degree in which these qualities are possessed is to some extent at least a 25 measure of the speed which can be attained in the use of a cutting tool and of the endurance of the cutting edge between sharpenings. The increase of the desirable qualities of alloys designed for such purposes 30 has therefore been constantly in view among metallurgists and heretofore a ternary alloy of cobalt, chromium and tungsten has been found to possess such desirable qualities in a high degree, the cobalt forming what may 35 be called the base of the alloy, or, as it may be called, a carrier for the other components, although the cobalt may be in relatively small proportion, and the chromium and tungsten, or perhaps the carbides thereof, in 40 alloy with the cobalt, giving the characteristic of hardness. In the development of the present invention it has been found that a ternary alloy of nickel, chromium and tungsten possesses the desirable quality of 45 mechanical strength to a higher degree than the alloy of cobalt, chromium and tungsten and to a higher degree than might have been expected from the results yielded by a binary alloy of nickel and chromium, although 50 the usefulness of nickel in known alloys in producing hardness and toughness has been known. Whether difficulties hitherto experienced in efforts to produce a satisfactory alloy of nickel, chromium and tungsten have prevented hitherto the production of such 55 an alloy is not known. In a co-pending application there is described a method by which such an alloy can be produced and in still another co-pending application there is described a method by which such an alloy 60 can be produced and in still another co-pending application is described a method of heat treatment by which the desirable qualities of such an alloy can be enhanced. 65 In the development of the present invention it has been found that the percentages of nickel, chromium and tungsten employed are of importance in producing the particular results desired. By way of example, two alloys designed for special purposes 70 may be described. 75 One of these alloys, designated as number 30 has an initial composition of 40% of tungsten, 40% of chromium and 20% of nickel, it being understood that by "initial" 80 composition it is intended to refer to the percentages of the several components with which the formation of the alloy is started, although, in the finished alloy, the percentages may differ more or less from various causes. It has been found that such an alloy, when properly alloyed and heat treated, 85 exhibits a hardness running from 90 to 100 on the scleroscope scale and a mechanical strength or toughness of about twice that of the specimens of the cobalt, chromium and tungsten alloy subjected to the same tests. It is found in practice that this alloy number 30 is not well adapted for intermittent cuts or for machining extremely tough 90 steel, such as heat treated chrome nickel steel, its mechanical strength, although greater than that of any alloy which approaches it in hardness, being insufficient for such duty. 95 The other alloy referred to and designated as number 9 has an initial composition of 15% of tungsten, 56% of chromium and 29% of nickel. This alloy, properly alloyed and heat treated, exhibits a very high degree 100 of mechanical strength. It is capable of taking very heavy feeds and cuts in metals

which cannot be cut commercially by other known alloys and stands up under interrupted or intermittent cuts, the shock of which will immediately break off the point of other alloy tools tested. Its hardness is such that it will wear several times as long as ordinary high speed steel and, having a high melting point, it will retain its hardness at cutting speeds two or three times the speed at which ordinary high speed steel will stand up. Because of its strength it can be used as a substitute for high speed steel in the majority of cases where such steel is used. It is not necessary to exercise caution in sharpening it to a blunt edge, since the mechanical strength is such that the edge can be brought to an angle considerably more acute than that which is ordinarily deemed possible, a lip angle of approximately 69%, for cutting cast iron, having been found successful.

Although it has been found thus far that chromium and tungsten in ternary alloy with nickel give highly satisfactory results, it is to be understood that other metals of the chromium group might be substituted for chromium and tungsten, in a ternary alloy.

Furthermore it will be understood that for the attainment of specific purposes it may be desirable under some circumstances to add certain quantities of other metals.

It will also be understood that other substances than those named may be used in making the alloy, to serve as purifiers, scavengers or fluxes.

Reference has been made above to the meaning of the expression "initial composition" and it will be understood that whatever may be the initial composition, the final composition of the finished alloy may differ considerably from the initial composition, by reason of variations in the method of forming the alloy or for other reasons. Thus more or less of the tungsten may be oxidized and carried off in the slag, together with the impurities in the commercial raw materials employed. Again, more or less of the nickel or chromium may be volatilized. The exercise of care in practicing the method of making the alloy, however, will enable substantially uniform results to be secured and it will be understood that variations within reasonable limits are not of themselves sufficient to change the characteristics of the finished tools beyond a commercial point. A statement of the exact final chemical analysis therefore cannot be offered as a determination of the characteristics of an alloy which embodies the invention. Another reason for the undesirability of depending upon a chemical analysis of the finished alloy lies in the fact that variations in the chemical composition of different parts of the tool may be caused

by the heat treatment so that chemical analysis of one part of a tool may differ from that of another part of the same tool.

Reference has been made above to the possibility of the hardness of the cobalt alloy being due in part to the presence of carbon in the form of carbides and it will be understood that the alloy which is the subject of the present application may also advantageously include a small percentage of carbon, whether added purposely or resulting from the working of the alloy in a graphite crucible.

It has been assumed, in the foregoing explanation of the nature of the invention, that the components used in making the alloy are used in their ordinary commercial state as to their purity, but it will be understood that they may be used as found in other combinations as, for example, Monel metal, which has a large content of nickel, might be used, in a suitable proportion, in place of the ordinary commercial nickel.

Reference has been made herein to the special suitability of the alloy for tools which are to be subjected to high duty in cutting of hard metals, but it will be understood that the alloy is well adapted for other uses which require either sharpness or a non-corrosive quality such as that possessed by the alloy described.

I claim as my invention:

1. An alloy of nickel in the proportion of not more than 30 and not less than 15 per cent of the whole and two metals of the chromium groups each present in a proportion of not less than 15 per cent of the whole and together forming not over 85 and not less than 70 per cent of the whole.

2. An alloy of nickel in the proportion of not more than 30 and not less than 15 per cent of the whole and chromium and another metal of the chromium group each present in a proportion of not less than 15 per cent of the whole and together forming not less than 70 and not over 85 per cent of the whole.

3. An alloy of nickel in the proportion of not more than 30 and not less than 15 per cent of the whole and chromium and tungsten each present in a proportion of not less than 15 per cent of the whole and together forming not less than 70 and not over 85 per cent of the whole.

4. An alloy of nickel in the proportion of not more than 30 and not less than 15 per cent of the whole chromium in a proportion of not less than 40 per cent and not over 60 per cent of the whole, and tungsten in a proportion of not less than 15 and not over 40 per cent of the whole, the chromium and tungsten together forming not less than 70 and not more than 85 per cent of the whole.

5. An alloy of nickel in the proportion of not more than 30 and not less than 15 per cent

cent of the whole and chromium and tungsten in equal proportions and together forming not less than 70 and not over 85 per cent of the whole.

6. An alloy of nickel in the proportion of not more than 30 and not less than 15 per cent of the whole two metals of the chromium group each present in a proportion of

not less than 15 per cent of the whole and together forming not over 85 per cent and 10 not less than 70 per cent of the whole and a relatively small percentage of carbon.

This specification signed this 19th day of January, A. D. 1924.

JEAN H. L. DE BATS.